

Dec. 19, 1922.

1,438,949.

J. DEAN.

METAL CHARACTER FOR PATTERNS.

FILED OCT. 24, 1921.

*Fig. 1.*



*Fig. 2.*



Witness:

Robert F. Becker

By

Hubert E. Peck Attorney

John Dean Inventor

Patented Dec. 19, 1922.

1,438,949

# UNITED STATES PATENT OFFICE.

JOHN DEAN, OF RACINE, WISCONSIN.

## METAL CHARACTER FOR PATTERNS.

Application filed October 24, 1921. Serial No. 509,864.

To all whom it may concern:

Be it known that I, JOHN DEAN, a citizen of the United States of America, and a resident of Racine, county of Racine, State 5 of Wisconsin, have invented certain new and useful Improvements in and Relating to Metal Characters for Patterns, of which the following is a specification.

This invention relates to certain improvements in metal characters or indicia for application or attachment to patterns employed in preparing molds for the production of metal castings; and the objects and nature of the invention will be readily understood 10 by those skilled in the art in the light of the following explanation of the accompanying drawings illustrating what I now believe to be the preferred mechanical expression or embodiment of my invention from among 15 other formations, constructions and combinations of metals and alloys within the spirit and scope thereof.

Those skilled in the pattern maker's art are familiar with the common brass and white 20 metal pattern letters and other characters of commerce. These characters are made of brass for metal patterns and are usually secured to such metal castings by the use of solder. The so-called white metal letters of 25 commerce are used for wood patterns and are usually secured thereto by shellac or other adhesive with or without the use of small brads. These white metal letters are usually composed of type metal or other 30 comparatively soft low melting point alloys. The white metal characters are not used on 35 metal patterns because they would not stand up under the hard usage to which such patterns are subjected in actual practice, and 40 because ordinary solder cannot be employed for securing such characters owing to the comparatively low temperature at which the 45 white metal characters melt. The brass pattern characters are expensive mainly because of the high melting point of brass and the consequent necessity of melting the metal in crucibles and casting the same in sand molds and the resulting excessive amount of handling and hand finishing work required to 50 individually prepare each separate character for the market.

It is an object of my invention to produce white metal or alloy pattern characters having a tight hard metal shell or jacket where- 55 by such characters can be produced at a com-

paratively low cost and can be successfully secured to and used on metal patterns.

With these and other objects in view, my invention consists in certain novel features in construction and in combination, as well as 60 in a novel and advantageous article, as more fully and particularly set forth and specified hereinafter.

Referring to the accompanying drawings;

Fig. 1 shows a pattern character in plan 65 view, and

Fig. 2 a cross section on the line 2—2, Fig. 1, the character being shown in the drawings on an enlarged scale for purposes of illustration.

Pattern characters—so-called letters—include not only letters and numerals, but also special marks, trade marks and various indications for attachment to patterns and consequent reproductions in the sand molds 70 and in the articles cast in such molds, all as will be understood by those skilled in the art. Hence, the term "characters" is herein employed in a broad generic sense to include all 75 indicia for attachment to patterns, and my invention is not limited to such indicia in the form of letters of the alphabet one of which I happen to illustrate for purposes of explanation.

The pattern character of my invention 80 consists of a soft or white metal body 1 completely encased and enclosed in a hard metal retaining jacket, shell or case 2. The metal body is preferably composed of a low 85 fusing point alloy that can be easily and inexpensively melted and produced in various forms by casting in metal molds or by any other suitable process. For this purpose I prefer to employ an alloy that does not expand when melted. For instance, a soft 90 metal low-fusing point alloy containing the necessary proportion of antimony possesses this non-shrinking characteristic, and I can employ tin, lead or zinc alloys containing 95 antimony in the proper proportion to cause the alloy to remain approximately the same 100 in size or bulk whether cold or melted.

Pattern indicia composed of this soft alloy 105 or other suitable material, are then encased in a tight impervious shell or jacket of copper, nickel or other suitable hard high fusing point metal in any suitable manner or by any suitable process, preferably by electrolysis or by any suitable method of depositing metal.

The soft metal pattern characters are first produced in finished condition and perfect form ready for use as wood pattern characters, i. e., for use on wood patterns. The 5 hard metal is then deposited on the surfaces of the finished complete soft metal character and forms a jacket exactly conforming to such surfaces and hence produces a perfect complete hard metal-exterior pattern character. The hard metal jacket forms an intimate part of the soft metal character, in effect an integral part thereof, and is impervious to serve as a container for the soft metal.

15 The encased characters can be secured to metal patterns by soldering even by the use of the ordinary solder which has a fusing point higher than that of the alloy of the characters. If the temperature employed in 20 soldering the characters is sufficiently high to fuse the soft metal of the characters, no difficulty results, as the copper (or other hard metal jacket) retains the alloy and maintains the proper form and shape of each 25 character.

The hard jacket protects the soft metal interiors against blows and rough usage, and hence my pattern characters can serve the purposes of the common solid cast brass 30 pattern letters, and yet can be produced at far less expense in the process of production as well as in raw material.

These soft metal filled hard metal encased letters and other characters are adapted for sign and other work where such characters 35 are secured to metal plates or other bodies by soldering.

What I claim is:

1. A pattern character consisting of a soft alloy body and a copper enclosing jacket. 40
2. A metal letter or other character for attachment to a metal body by soldering, consisting of a soft low-fusing point body, and a high fusing point hard metal retaining jacket completely enclosing said body. 45
3. A pattern character consisting of a body composed of a low fusing point alloy that includes antimony as an ingredient, and an exterior high fusing point hard metal jacket completely encasing said body. 50
4. A pattern character comprising a body composed of a low fusing point non-expanding alloy, and a high fusing point protecting and retaining jacket enclosing said body. 55
5. As a new article of manufacture, a metal pattern character provided with and completely encased by a hard metal protecting and retaining jacket.
6. A pattern character consisting of a body composed of low fusing point metallic material provided with and encased by a hard metal retaining jacket forming the exterior finish of the character. 60

JOHN DEAN.